

G. PRIFOLD,  
WATERPROOF FLOOR COVERING,  
APPLICATION FILED FEB. 13, 1913.

1,176,853.

Patented Mar. 28, 1916.

*Fig. 1*



*Fig. 2*



Witnesses:  
M. E. Echard  
L. E. Johnston

George Prifold Inventor  
By his Attorneys  
Franklin & Associates

# UNITED STATES PATENT OFFICE.

GEORGE PRIFOLD, OF LINWOOD, PENNSYLVANIA, ASSIGNOR TO BARRETT MANUFACTURING COMPANY, OF NEW YORK, N. Y., A CORPORATION OF WEST VIRGINIA.

## WATERPROOF FLOOR-COVERING.

1,176,853.

Specification of Letters Patent. Patented Mar. 28, 1916.

Application filed February 13, 1913. Serial No. 748,080.

To all whom it may concern:

Be it known that I, GEORGE PRIFOLD, a citizen of the United States, residing in Linwood, county of Delaware, and State of Pennsylvania, have invented new and useful Improvements in Waterproof Floor-Coverings, of which the following is a specification.

This invention relates to improvements in flexible water-proof coverings composed of felt particularly, and has for its object the production of a felt covering for floors which shall serve as a substitute for so-called linoleum or oil-cloth and the like, and which is extremely cheap yet resistant to the ordinary wear and tear to which floor coverings are ordinarily subjected.

My investigations and experiments have led to the discovery that a covering of the above nature suitable for application to pitch-impregnated felt can be obtained by applying to a foundation of so-called wool felt saturated with a suitable pitchy water-proof composition, as for example asphalt, a priming coat consisting of a colloidal, organic glutinous material preferably soluble casein, which is combined with an inorganic, relatively non-absorbent, inert filler such as pulverized shale, or other minerals or materials which are relatively hard and non-porous and of an aluminiferous nature. To a felt primed with the foregoing mixture is applied a color or finish coat of a paint or a varnish and this when dried is preferably printed in the usual manner employed for printing linoleum or oil-cloth to produce any desired pattern or color effect thereon.

The preferred composition which I employ, although obviously various compositions may be employed without departing from the invention set forth in the accompanying claims, consists of a solution of one pound of soluble casein, such for example as is known in the trade as "Shac Lac Glue" in six pounds of water. This solution is allowed to stand first in the cold without heating for a half hour or hour and is then heated to thoroughly dissolve in so far as possible the said soluble casein. To this mixture is then added six pounds of finely powdered shale, such for example as is known in the trade as "Talckene," this

mixture having a composition of approximately the following:

|                   |        |    |
|-------------------|--------|----|
| Water             | 3.65%  | 55 |
| Silica            | 63.20% |    |
| Alumina           | 16.04% |    |
| Peroxid of iron   | 10.25% |    |
| Lime              | 0.59%  | 60 |
| Magnesia          | 3.02%  |    |
| Potash            | 2.50%  |    |
| Soda              | 0.65%  |    |
| Oxid of manganese | Trace  |    |
|                   | 99.90% | 65 |

This priming mixture is applied to the felt and allowed to thoroughly dry, and then any suitable paint or varnish, either with or without pigment, is applied thereover, for example a mixture consisting of one part linseed oil and two parts of gloss oil mixed with a pigment such as French ocher if desired, and thinned sufficiently with naphtha to the proper consistency for convenient application. A second coat consisting of one part linseed oil and two parts of varnish, together with any suitable pigment such as yellow ocher may be superposed upon the first color coat if desired. Then as stated the surface is printed or suitably impressed or embossed so as to produce any desired color effects or pattern thereon in imitation of oil-cloth or linoleum.

In the accompanying drawing, forming part of this specification, Figure 1 illustrates a cross section of my improved floor covering showing the successive layers or steps of my process, and Fig. 2 is a plan view of the same.

The portion 2 represents the base or foundation of felt, 3 the priming coat, 4 the oil and varnish coating, and 5 the decorating or embossing to give the final ornamental finish.

The priming coat is not only adhesive both to the foundation layer and to the color coating, but is also resistant to the pitch-like impregnating compositions of the felt and to the oils, and alcoholic and other ingredients contained in the finish coating. Moreover, because of the presence of an inorganic water-insoluble, non-absorbent filler, such as the pulverized shale, the coating of paint

or varnish applied thereto is not only prevented from being absorbed into the felt, but is rendered much harder than is the case where a water soluble inorganic salt is employed, since said water insoluble filler acts as an abrasive and serves to augment the hardness of the paint or color coating.

A floor covering prepared in accordance with the foregoing illustration can be flexed 10 without noticeable cracking, and has all of the durable properties of an expensive coated linoleum fabric, since the felt foundation is sufficiently elastic to permit of the yielding impact of the paint or varnish coat 15 against the shoe of the wearer or the tire of a vehicle, such as a truck or the like, which may come in contact therewith in the ordinary use within buildings and the like.

The term "pitchy" or "pitch-like" as 20 employed in the claims includes "pitchy materials" generically, including pitch obtained by the distillation of turpentine, bitumen or asphalt, as well as petroleum pitches, coal tar pitches or like materials 25 treated to impart pitch-like properties thereto.

This invention is distinguished from the invention set forth in the patent to J. Smith, No. 1,008,296 of November 7, 1911 for waterproof floor covering, assigned to the Barrett Manufacturing Company, the assignee of this application, in that the Smith invention comprises the employment of an inorganic colloidal glutinous material as one of the essential elements of the composition.

My invention on the other hand does not include the use of such a composition and the same is hereby disclaimed, but it does specifically include the use of a sizing coating of water-soluble organic glutinous material in conjunction with a water-insoluble mineral filler and the other elements set forth in the claims appended hereto.

Having thus described my invention, what 45 I claim and desire to secure by Letters Patent is:—

1. A water-proof covering for floors and the like, comprising a so-called wool felt foundation impregnated with a water-proof-

ing composition, of a pitch-like nature, a 50 coating of sizing superficially applied thereto, said sizing including a water soluble colloidal organic albuminous material and a pulverized shale mineral filler and a finish coating containing paint or varnish super- 55 posed upon said sizing coating, said sizing coating being adhesive to both said foundation and said finish coating, and being also resistant to the impregnating composition of said foundation and the ingredients of 60 said finish coating.

2. A water-proof covering for floors and the like, comprising a soluble wool felt foundation impregnated with a water-proofing composition, of a pitch-like nature, a coating 65 of sizing superficially applied thereto, said sizing including a water-soluble colloidal organic albuminous material and a relatively non-porous pulverulent mineral filler and a finish coating containing paint 70 or varnish superposed upon said sizing coating, said sizing coating being adhesive to both said foundation and said finish coating, and being also resistant to the impregnating composition of said foundation and 75 the ingredients of said finish coating.

3. A waterproof covering for floors and the like, comprising a soluble wool felt foundation impregnated with a water-proofing composition, of a pitch-like nature, a coating 80 of sizing superficially applied thereto, said sizing including a casein material and a relatively non-porous pulverulent mineral filler and a finish coating containing paint or varnish superposed upon said sizing coating, said sizing coating being adhesive to both said foundation and said finish coating, and being also resistant to the impregnating composition of said foundation and the ingredients of said finish coating.

In witness whereof, I have hereunto set my hand at Linwood, aforesaid, this 12 day of February, 1913.

GEORGE PRIFOLD.

Witnesses:

GEORGE E. APPLEBY,  
FRANK B. FOSTER.